

[54] FLUORINATED ALIPHATIC  
POLYALKYLETHER LUBRICANT WITH AN  
ADDITIVE COMPOSED OF AN AROMATIC  
PHOSPHINE SUBSTITUTED WITH  
PERFLUOROALKYLETHER GROUPS

[75] Inventors: Carl E. Snyder, Jr., Trotwood; Christ  
Tamborski, Dayton, both of Ohio

[73] Assignee: The United States of America as  
represented by the Secretary of the  
Air Force, Washington, D.C.

[21] Appl. No.: 417,931

[22] Filed: Sep. 14, 1982

[51] Int. Cl.<sup>3</sup> ..... C10M 1/30; C10M 1/44

[52] U.S. Cl. ..... 252/49.9; 252/54;  
252/389 A

[58] Field of Search ..... 252/49.9, 54, 389 A

[56] References Cited

U.S. PATENT DOCUMENTS

|           |         |                  |             |
|-----------|---------|------------------|-------------|
| 3,306,855 | 2/1967  | Borecki          | 252/49.9    |
| 3,393,151 | 7/1968  | Dolle et al.     | 252/49.9    |
| 3,481,872 | 12/1969 | Dolle et al.     | 252/49.9    |
| 3,483,129 | 12/1969 | Dolle et al.     | 252/49.9    |
| 3,499,041 | 3/1970  | Tamborski        | 260/612     |
| 3,567,802 | 3/1971  | Garth            | 260/950     |
| 4,011,267 | 3/1977  | Tamborski et al. | 260/606.5 P |

4,043,926 8/1977 Snyder et al. .... 252/49.9  
4,097,388 6/1978 Snyder et al. .... 252/49.9

Primary Examiner—Jacqueline V. Howard  
Attorney, Agent, or Firm—Donald J. Singer; Charles E.  
Bricker

[57]

ABSTRACT

A lubricant composition comprising a base fluid having the general formula



wherein n is an integer, and a corrosion inhibiting amount of an aromatic phosphine with perfluorinated polyalkylether substituents having the general formula



wherein  $R_jOR_j$ — is a perfluoroalkylether group containing at least one ether linkage.

10 Claims, No Drawings

**FLUORINATED ALIPHATIC POLYALKYLETHER LUBRICANT WITH AN ADDITIVE COMPOSED OF AN AROMATIC PHOSPHINE SUBSTITUTED WITH PERFLUOROALKYLETHER GROUPS**

**RIGHTS OF THE GOVERNMENT**

The invention described herein may be manufactured and used by or for the Government of the United States for all governmental purposes without the payment of any royalty.

**BACKGROUND OF THE INVENTION**

This invention relates to lubricating compositions. Because of their thermal stability, perfluorinated polyalkylether fluids have great potential for use as engine oils, hydraulic fluids and greases. However, a serious drawback in their use results from the fact that certain metals, i.e., those likely to be present in aircraft engine components, are corroded by these fluorinated fluids at elevated temperatures in an oxidative environment. For example, when the fluids are utilized as lubricants for mechanical components composed of mild steels, serious corrosion has occurred at temperatures of about 550° to 600° F. Stainless steels, titanium and titanium alloys are attacked by the fluids at a temperature of about 600° F. Moreover, at elevated temperatures, particularly in an oxidizing atmosphere, the fluids themselves undergo considerable degradation, to the detriment of continued lubricating capacity.

An ideal lubricant composition would be one having a relatively constant viscosity such that it is flowable or pumpable over a wide temperature range, e.g., from about -50° F. to about 600° F. In general, base fluids available heretofore have either had a satisfactory viscosity at low temperatures, but degraded at elevated temperatures, or, were stable and had a satisfactory viscosity at elevated temperatures, but were too viscous to flow or pump at subzero temperatures. Consequently, it has been necessary to make compromises in the selection of base fluids dependent upon the use conditions to be encountered. Such compromises have not been entirely satisfactory.

In U.S. Pat. No. 3,393,151, issued to one of us as a coinventor on July 16, 1968, lubricants are disclosed that comprise a perfluorinated aliphatic polyether and a perfluorophenyl phosphorus compound. In U.S. Pat. No. 3,499,041, issued to one of us on March 3, 1970, certain perfluoroaryl phosphines are disclosed as being anticorrosion additives for perfluorinated fluids. In U.S. Pat. No. 3,483,129, issued to one of us as a coinventor on Dec. 9, 1969, certain perfluorinated phenoxyphenyl phosphines are disclosed as being anticorrosion additives for perfluorinated fluids. In U.S. Pat. No. 3,567,802, certain perfluoropolyoxoalkane-substituted phosphines are disclosed as being useful as corrosion and degradation inhibitors for perfluorinated fluids. In U.S. Pat. No. 4,011,267, issued to use as coinventors on Mar. 8, 1977, certain fluorinated phosphines are disclosed as being anticorrosion and antioxidant additives for perfluorinated fluids. While the phosphorus compounds described in these patents exhibit corrosion inhibiting properties, at low temperatures most of these compounds are only poorly soluble in fluorinated fluids. Also, certain members of the classes of phosphorus compounds possess high volatility characteristics for long term high temperature applications. Because of these limitations, fluorinated fluids containing such anti-

corrosion additives are not completely satisfactory for use in long term, wide temperature range applications.

It is an object of this invention to provide a lubricant composition which has little if any corrosive effect upon ferrous alloys.

Another object of this invention is to provide a lubricant composition which has a relatively constant viscosity over a wide temperature range.

Other objects and advantages of the invention will be apparent to those skilled in the art upon consideration of the following disclosure.

**SUMMARY OF THE INVENTION**

In accordance with the present invention there is provided a lubricant composition comprising (1) a base fluid consisting essentially of a mixture of fluorinated polyethers having the following formula:



wherein n is an integer indicating the degree of polymerization, and (2) a corrosion inhibiting amount of an aromatic phosphine with perfluorinated polyalkylether substituents having the general formula:



wherein  $R_1OR_2$ — is a perfluoroalkylether group containing at least one ether linkage. Examples of  $R_1OR_2$ — groups include the following:



where x, y and z are zero or an integer having a value of 1 to 20, preferably 1 to 4, inclusive. A detailed description of the synthesis of these phosphine compounds is contained in application Ser. No. 418,155, filed of even date herewith by C. Tamborski, C. E. Snyder, Jr., and J. B. Christian, the disclosure of which is incorporated herein by reference. The preferred phosphines are those in which the perfluoroalkylether group is para to the phosphorus atom.

The base fluid may be one or more of a homologous series of hydrogen-containing fluorinated ethers. These fluids are prepared from hexafluoropropylene oxide and have the general structural formula given previously. A series of such hexafluoropropyl ethers is available from the "Freon" Products Division of E. I. duPont de Nemours and Company, Wilmington, Del., which manufactures and sells the same under the tradename "Freon E". In the presently available series of "Freon E" fluids, the number in the name corresponds to the average n in the formula. Thus, any particular homolog such as Freon E-7 can vary in the composition of its mixture so long as the average n corresponds to the number in its name.

In formulating the lubricant of this invention, a corrosion-inhibiting amount of the phosphine compound is mixed with the fluorinated polyether base fluid. The amount of the phosphine used generally ranges from

0.05 to 5 weight percent, preferably 0.5 to 2 weight percent, based upon the weight of the base fluid.

The following example illustrates the invention.

#### EXAMPLE

A series of runs was conducted for the purpose of determining the effectiveness of lubricant compositions of this invention. Lubricant compositions were formulated by mixing (1) Freon E-7 base fluid and (2) a fluorinated phosphine having the following formula:



In the runs, specimens of steel were immersed in the formulations that were prepared. The compositions of the steels are described in the literature. For comparison purposes, runs were carried out in polyether fluid which did not contain the phosphine additive. The materials were contained in an oxidation test tube having a take-off adapter coupled to an air entry tube. An aluminum block both provided the means for heating the test tube and an "overboard" test procedure (no reflux condenser) was followed.

Air was bubbled through the materials at the rate of 1 liter of air per hour for a period of 24 hours. The runs were conducted at temperatures ranging from 500° to 650° F. The specimens and the apparatus were weighed before and after each run.

The data obtained in the runs are set forth below in the table.

TABLE I

| Temperature (°F.)               | 500   | 25    | 600   | 625   | 650   |
|---------------------------------|-------|-------|-------|-------|-------|
| Wt % additive                   | 0     | 0     | 1.0   | 1.0   | 1.0   |
| Kinematic Viscosity             | +4.79 | +8.0  | +6.12 | +2.45 | +2.50 |
| Change at 100° F., %            |       |       |       |       |       |
| Fluid Loss Wt %                 | 2.90  | 16.5  | 2.38  | 1.11  | 2.91  |
| Acid Number Increase            | 6.45  | 7.93  | 0.11  | 0.07  | 0.31  |
| mgKOH/g                         |       |       |       |       |       |
| Wt Change in mg/cm <sup>2</sup> |       |       |       |       |       |
| 4140 Steel                      | +0.11 | -2.72 | +0.07 | +0.04 | +0.22 |
| 52100 Bearing Steel             | +0.11 | -1.28 | +0.05 | +0.03 | +0.23 |
| 410 Stainless Steel             | -0.22 | -4.53 | +0.02 | +0.04 | +0.05 |
| M-50 Tool Steel                 | +0.16 | -2.41 | +0.05 | +0.03 | +0.02 |
| 440 C. Stainless Steel          | 0.88  | -5.14 | +0.03 | -0.01 | 0.00  |

The data in the foregoing table show that the lubricant compositions of the invention have little, if any, corrosive effect upon ferrous alloys. Also, there was substantially no degradation of the lubricant compositions at the elevated temperatures even though the base fluid without the additive was severely degraded. Due to the nearly complete degradation and subsequent loss of the base fluid above 525° F. in the presence of ferrous alloys, it was not possible to provide comparative data at those temperatures. Because of their outstanding properties, the lubricants of this invention can be employed for applications requiring extreme temperature

conditions. Thus, the lubricants of this invention may be employed, for example, as gas turbine engine lubricants, nonflammable hydraulic fluids greases compatible with liquid oxygen, liquid coolants and general purpose lubricants.

Various modifications may be made in the present invention without departing from the spirit of the invention or the scope of the following claims.

We claim:

1. A lubricant composition comprising (1) a base fluid consisting essentially of a fluorinated polymer having the formula



wherein n is an integer indicating the degree of polymerization and (2) a corrosion inhibiting amount of an aromatic phosphine with perfluorinated polyalkyether substituents having the formula



wherein  $\text{R}_1\text{OR}_2-$  is a perfluoroalkylether group containing at least one ether linkage.

2. The composition of claim 1 wherein the amount of said phosphine ranges from about 0.05 to 5 weight percent.

3. The composition of claim 1 wherein the amount of said phosphine ranges from about 0.5 to 2 weight percent.

4. The composition of claim 1 wherein said  $\text{R}_1\text{OR}_2-$  in said phosphine is



wherein x is zero or an integer having a value of 1 to 20.

5. The composition of claim 4 wherein said x is in the range of 1 to 4.

6. The composition of claim 4 wherein said x is 1.

7. The composition of claim 1 wherein said  $\text{R}_1\text{OR}_2-$  in said phosphine is



wherein y is zero or an integer having a value of 1 to 20.

8. The composition of claim 7 wherein said y is in the range of 1 to 4.

9. The composition of claim 1 wherein said  $\text{R}_1\text{OR}_2-$  in said phosphine is



wherein z is zero or an integer having a value of 1 to 20.

10. The composition of claim 9 wherein said z is in the range of 1 to 4.

\* \* \* \* \*

UNITED STATES PATENT AND TRADEMARK OFFICE  
CERTIFICATE OF CORRECTION

PATENT NO. : 4,443,349

DATED : Apr 17, 1984

INVENTOR(S) : Carl E. Snyder, Jr., Christ Tamborski

It is certified that error appears in the above-identified patent and that said Letters Patent is hereby corrected as shown below:

Column 3, Table I, the first entry in numerical column 2 which now reads "25" should read -- 525 --.

Claim 1, line 2, "polymer" should read -- polyether --.

**Signed and Sealed this**

*Eighteenth Day of September 1984*

**[SEAL]**

*Attest:*

**GERALD J. MOSSINGHOFF**

*Attesting Officer*

*Commissioner of Patents and Trademarks*